

1,372,483.

C. G. COLLINS.  
PROCESS FOR THE REDUCTION OF ORES.  
APPLICATION FILED MAR. 26, 1920.

Patented Mar. 22, 1921.

2 SHEETS—SHEET 1.



FIG. 1.

INVENTOR

Caleb G. Collins  
BY  
Wm Wallace White  
ATTORNEY

C. G. COLLINS,  
PROCESS FOR THE REDUCTION OF ORES,  
APPLICATION FILED MAR. 26, 1920.

1,372,483.

Patented Mar. 22, 1921.

2 SHEETS—SHEET 2.



INVENTOR

Caleb G. Collins  
BY  
Wallace Whit  
ATTORNEY

# UNITED STATES PATENT OFFICE.

CALEB G. COLLINS, OF WOODMERE, NEW YORK, ASSIGNOR TO C. AMORY STEVENS, OF NEW YORK, N. Y.

## PROCESS FOR THE REDUCTION OF ORES.

1,372,483.

Specification of Letters Patent. Patented Mar. 22, 1921.

Application filed March 26, 1920. Serial No. 368,973.

To all whom it may concern:

Be it known that I, CALEB GROZIER COLLINS, a citizen of the United States, residing at Woodmere, county of Nassau, State of

5 New York, have invented new and useful Improvements in Processes for the Reduction of Ores, of which the following is a specification.

My invention has for its object the reduction of ores, and while applicable in a general way, is particularly adapted to the extraction of aluminum from ores containing alumina, reducing at the same time, however, the other metals in the ore.

10 The invention consists in a process for the extraction of ores involving the mixture of sodium chlorid, with the ore and with a carboniferous substance with or without the addition of oxalates formed preferably by 15 the inclusion of sawdust impregnated with alkali in the mixture. The addition of the oxalates assists materially in obtaining higher yields, and at lower temperatures. The particular advantages in the use of 20 sawdust to produce the oxalates, rather than adding oxalates directly to the mixture, are 25 that the chlorin is set free from the sodium chlorid, and sets the oxalates free from the mixture so that the oxalates are formed in 30 nascent state, and also that the carbon of the sawdust is an aid to the reduction of the ore.

In order that my process may be clearly set forth and easily understood, I have illustrated in the accompanying drawings a preferred form of furnace in which the process may be carried out; and in describing the process, reference will be made to these drawings, it being understood that my invention resides in the process itself, the particular form of apparatus used in carrying it out being immaterial.

40 In these drawings, Figure 1 shows a furnace in vertical section approximately on the line 1—1 of Fig. 2, and Fig. 2 is a vertical section taken approximately on the line 2—2 of Fig. 1.

The furnace comprises a number of ore chambers, 1, 2, 3. These are preferably 45 closed by walls 4 of fire brick, inclined so as to form an ore chamber tapering from a narrow opening at the top to a greater width at the bottom to facilitate the passage of the ore. The walls 4 of adjacent ore chambers

are spaced to provide passages 5 for the furnace gases for heating the ore, and spaces 6 at the lower parts for cooling the ore before removal.

Heat is provided by a fire on the grate 7 disposed in a fire box 8 arranged along the ends of the ore chambers. The gases pass through openings 9 into the heat passages 5 between the ore chambers, and between the end ore chambers and the walls 10 of the furnace, and pass upward through the passages 5, being guided over a lengthy path by baffles 11 to afford opportunity for the heat to be transmitted to the ore before the gases reach the stacks 12. As the gases still retain some heat as they pass up the stacks, 70 they are led by a conducting pipe 13 into a preheating device 14 where they pass around a container 15 and escape by the chimney 16.

The ore mixture is fed to the furnace by a 75 hopper 17 which discharges into the pre-heating container 15. This container is preferably rotatably mounted and slightly inclined, so that the ore is heated as it passes through, and emerges at the other end, being 80 guided by a chute 18 into a hopper 19, having individual hoppers 20 leading to the several ore chambers. In order to distribute the ore mixture evenly to the several individual hoppers 20, the ore from the chute 85 18 strikes a guide plate 21. The apparatus 90 should be operated at such a rate as to always keep the ore chambers full, and thereby prevent access of air, gases formed in the chambers however being permitted to escape by percolating up through the ore mixture in the hoppers.

As the ore passes down through the ore chambers, it receives heat through the walls, and the treatment of the ore takes place, 95 until the ore passes below the line of the separating baffles or walls 22 which separate the heating chambers 5 from the cooling chambers 6, whereupon the treated ore commences to cool down, and is removed, preferably by means of a screw conveyer 23 which draws the ore out and discharges it into a receiving chamber 24 from which it may be removed at will. The speed of operation may be controlled by the conveyer 100 screw 23 and a device including a drum 25 provided with a plurality of buckets or vanes 26 which is rotatably mounted just

above the conveyer, and serves to break up the ore and keep it moving at a uniform rate.

The process as carried out in the form of apparatus shown consists in first reducing to a comminuted state, preferably from 20 to 40 mesh, according to the hardness of the ore, and mixing, the ore, a material containing carbon, and sodium chlorid, which are fed into the hopper 17. To this mixture may be added oxalates. In place of adding oxalates in their ordinary commercial form, I prefer to use sawdust, impregnated with soda or other alkalis.

This mixture passes through the preheater and into the chambers 1, 2, 3, the ore mixture in the hoppers preventing access of air to the interior during the heating operations, and the furnace is fired to produce a heat within the chamber preferably in the neighborhood of 1400° Fahrenheit. Since the apparatus is arranged for continuous operation, the length of time for heating to complete the reduction may be regulated by controlling the speed of operation of the devices for breaking and removing the treated ore, so that by the time the ore reaches the level of the cooling chambers, the reduction will be complete, and the product may be removed.

The proportions of sodium chlorid and sawdust naturally vary with the particular ore being treated, but in general the quan-

35  
tity of carbon may be about 5% of the quantity of ore, the sodium chlorid about 3% and the sawdust impregnated with alkali about 2%.

Having now described my invention I claim and desire to secure by Letters Patent:

1. The process of reducing aluminum from ores which consists in comminuting and mixing the ore, a carboniferous material, and sodium chlorid, subjecting the mixture to heat, and preventing access of air to the mixture during the heating.

40  
2. The process of reducing aluminum from ores which consists in comminuting the ores, and treating them under the influence of heat and while preventing access of air, with carboniferous material, sodium chlorid, 45 and oxalates.

3. The process of reducing aluminum from ores which consists in comminuting and mixing the ore, sawdust previously impregnated with alkali and sodium chlorid, 50 and subjecting the mixture to heat while preventing access of air.

4. The process of reducing aluminum from ores which consists in comminuting, and mixing the ore, carboniferous material, 60 sawdust previously impregnated with alkali, and sodium chlorid, and subjecting the mixture to heat while preventing access of air.

In testimony whereof I have signed my name to this specification.

CALEB G. COLLINS.